# EUROPEAN PATENT SPECIFICATION

(11) **EP 2 520 709 B1**
(45) Date of publication and mention of the grant of the patent: **30.03.2016**
(21) Application number: 12167036.8
(22) Date of filing: 07.05.2012
(51) Int. Cl.: D21H 13/00, D21H 19/40, D21H 19/82

(54) **Sand-effect paper material and corresponding manufacturing method**
Sandeffektpapiermaterial und entsprechendes Herstellungsverfahren
Structure cellulaire pour panneau à double courbure

(30) Priority: 06.05.2011 IT MI20110779
(43) Date of publication of application: 07.11.2012
(73) Proprietor: GRUPPO CORDENONS S.p.A., 20145 Milano (IT)
(72) Inventor: Monacelli, Luca, 33170 Pordenone (IT); Gilberti, Ferruccio, 20121 Milano (IT)
(74) Representative: Rapisardi, Mariacristina

(56) References cited:
- EP-A2- 1 762 656
- WO-A1-00/22231
- DE-A1- 4 118 340
- DE-A1- 19 706 574
- US-A- 5 334 286

## Description

### "SAND-EFFECT PAPER MATERIAL AND CORRESPONDING MANUFACTURING METHOD"

The present invention relates to a sand-rough-effect paper material (paper/cardboard) and to the corresponding manufacturing method. More precisely, the paper material of the invention, thanks to an appropriately devised pulp and to a specific surface treatment, loses the typical feel of paper materials and is characterized by a feel similar to that of sand.

US 5334286 A and WO 00/22231 A1 disclose a tissue-type paper material, not suitable for printing with high quality.

In the paper-making sector there is a constant search for new types of papers having particular appearances and/or finishes, above all designed for wrapping, packaging, production of illustrative material, quality printing, etc.

Not infrequently, however, these particular effects are achieved at the expense of other characteristics of the paper, for example, printability.

An aim of the present invention is to provide a paper material that presents a feel different from that of traditional paper materials and at the same time enables a high printing quality.

The present invention hence regards a paper material and the corresponding manufacturing method as defined in the annexed Claims 1 and 7, respectively.

Preferred embodiments of the paper material and of the corresponding manufacturing method are defined in the dependent Claims.

The invention hence provides a sand-effect paper material (paper/cardboard), which, thanks to an appropriately devised pulp and to a specific surface treatment, loses the typical feel of paper materials and is characterized by a feel similar to that of sand, having a rough surface finish typical of a surface covered with fine sand.

The paper material of the invention moreover ensures a high printing quality and enables particular graphic effects to be achieved, which are difficult to obtain with traditional coated papers.

In detail, the paper material of the invention comprises a substrate that is formed by a mixture of cellulose fibres and contains at least one polymeric substance, capable of bestowing (dry and wet) strength on the mixture of fibres, and an inorganic filler, capable of bestowing on the material good characteristics of machinability.

The substrate has at least one surface (face) treated with at least one surface adhesive and a glossy coating having particular components so that the paper material, owing to the combined effect of the composition of the substrate and of the surface treatment, presents a feel similar to that of sand. Clearly, both of the faces of the substrate can be treated in the same way.

Preferably, the polymeric substance included in the substrate comprises one or more colophony-based and/or alkyl-ketene-dimer-based and/or acetyl-succinic-acid-based and/or epichlorohydrin-based resins, and/or modified starches, and the inorganic filler is a mineral filler comprising one or more substances selected in the group consisting of carbonates, kaolins, talc, and mixtures thereof.

The surface adhesive is, for example, an adhesive with a base of starch and/or polyvinyl alcohol and/or acrylic, polyurethane and/or styrene-butadiene polymers. Moreover, the paper material of the invention is provided with a glossy coating, applied on the treated surface (clearly, the paper material can have both of the surfaces treated and provided with a glossy coating).

In particular, the glossy coating is formed by one or more binding polymers (for example, polyurethane-based and/or silicone-based polymers, and/or acrylic polymers, styrene-butadiene polymers, polyvinyl-acetate polymers, polyvinylalcohol polymers, and the like) and/or waxes, mixed with pigments, for example, pigments with a lamellar or flat structure, such as, for example, precipitated calcium carbonate (PCC), kaolins for coating, calcined and/or lamellar kaolins, in combination with pigments with a base of calcium silicates having different grain sizes and degree of whiteness higher than 85 (according to the DIN 5033 standard).

These calcium-silicate-based pigments, preferably having particles of variable grain size and a particular degree of whiteness are especially important for achieving the desired effect.

In particular, the pigments comprise wallastonite (calcium silicate of formula CaSiO₃).

The amount of polymer per face is preferably comprised between 5% and 100% with respect to the pigments; the substance of the paper material is comprised between 90 g/m² and 350 g/m²; the amount of glossy coating spread on each face is comprised between 5 g/m² and 20 g/m².

The glossy coating may be coloured and/or spread on a coloured substrate; preferably, colours in paste form and organic or inorganic pigments are used.

The paper material just described is obtained, in accordance with a further aspect of the present invention, with the method described below.

First the substrate is provided with techniques of formation of paper that are substantially known, for example, on a paper machine.

Basically, an aqueous pulp is provided constituted by cellulose fibres, said pulp containing the polymeric substance (colophony-based and/or alkyl-ketene-dimer-based and/or acetyl-succinic-acid-based and/or epichlorohydrin-based resins, and/or modified starches) and the inorganic filler (carbonates, kaolins, talc, etc.).

Next, water is removed from the pulp to form the substrate of the paper material.

This is followed by a step of surface treatment of one or both of the faces of the substrate with an aqueous solution of surface adhesive, for example, made up of an aqueous solution of starch (10 wt%), and/or acrylic adhesive (5 wt%), or adhesives similar to the ones described previously (adhesives with a base of polyvinyl alcohol and/or of acrylic, polyurethane and/or styrene-butadiene polymers).

The treatment with the surface adhesive has also the purpose of bestowing on the paper material a correct penetration of water, indispensable for the subsequent coating step.

The method then comprises, after the surface treatment with adhesive, a step of smoothing of the substrate, where the substrate is smoothed up to Bendsten ISO 2494 roughness values of less than 50 ml/min and preferably of less than 30 ml/min, and indicatively 20 ml/min.

Next, the glossy coating described above is applied.

Preferably, application of the glossy coating is performed by spreading carried out with an air-blade or smoothing-blade coating machine, and is followed by a step of drying of the coating, conducted in an infrared oven and/or hot-air oven at a temperature of between 100°C and 180°C and with an oven time of between 0.5 and 4 minutes.

Finally, the method comprises a step of mechanical treatment of the surface provided with the coating, in particular a smoothing step and/or an embossing step.

## Claims

1. A sand-rough-effect paper material, comprising a substrate, formed by a mixture of cellulose fibres containing at least one polymeric substance, apt to bestow strength on the mixture of fibres, and an inorganic filler; and having at least one surface treated with at least one surface adhesive and provided with a glossy coating formed by one or more binding polymers and/or waxes, mixed with pigments; and wherein the pigments comprise pigments with a base of calcium silicate so that the paper material has a sand-like rough feel, the calcium-silicate-based pigments having variable grain size and degree of whiteness higher than 85 according to the DIN 5033 standard.

2. The paper material according to Claim 1, wherein the polymeric substance included in the substrate comprises one or more colophony-based and/or alkyl-ketene-dimer-based and/or acetyl-succinic-acid-based and/or epichlorohydrin-based resins, and/or modified starches.

3. The paper material according to Claim 1 or Claim 2, wherein the inorganic filler is a mineral filler and comprises one or more substances selected in the group consisting of carbonates, kaolins, talc, and mixtures thereof.

4. The paper material according to any one of the preceding claims, wherein the surface adhesive is an adhesive with a base of starch and/or polyvinyl alcohol and/or acrylic, polyurethane and/or styrene-butadiene polymers.

5. The paper material according to any one of the preceding claims, wherein the glossy coating comprises pigments with a lamellar or flat structure, such as, for example, precipitated calcium carbonate (PCC), kaolins for coating, calcined and/or lamellar kaolins, in combination with the calcium-silicate-based pigments.

6. The paper material according to any one of the preceding claims, wherein the binding polymers comprise polyurethane-based, acrylic-based, polyvinyl-alcohol-based, styrene-butadiene-based and/or silicone-based polymers.

7. A method for manufacturing the paper material according to any one of the preceding claims, comprising the steps of:
(a) preparing an aqueous pulp of cellulose fibres containing at least one polymeric substance, apt to bestow strength on the mixture of fibres, and an inorganic filler;
(b) removing water from the pulp to form a substrate of the paper material;
(c) treating at least one surface of the substrate with at least one surface adhesive in such a way as to bestow on the substrate characteristics of water penetration suitable for a subsequent coating step; and
(d) applying to the surface treated a glossy coating formed by one or more binding polymers and/or waxes, mixed with pigments comprising calcium-silicate-based pigments so that the paper material has a sand-like feel, wherein the calcium-silicate-based pigments have variable grain size and degree of whiteness higher than 85 according to the DIN 5033 standard.

8. The method according to Claim 7, wherein the polymeric substance included in the substrate comprises one or more colophony-based and/or alkyl-ketene-dimer-based and/or acetyl-succinic-acid-based and/or epichlorohydrin-based resins, and/or modified starches.

9. The method according to Claim 7 or Claim 8, wherein the inorganic filler is a mineral filler and comprises one or more substances selected in the group consisting of carbonates, kaolins, talc, and mixtures thereof.

10. The method according to any one of Claims 7 to 9, wherein the surface adhesive is an adhesive with a base of starch and/or polyvinyl alcohol and/or acrylic, polyurethane and/or styrene-butadiene polymers.

11. The method according to any one of Claims 7 to 10, wherein the glossy coating comprises pigments with a lamellar or flat structure, such as, for example, calcium carbonate, precipitated calcium carbonate (PCC), calcined and/or lamellar kaolins, kaolins for coating in combination with the calcium-silicate-based pigments.

12. The method according to any one of Claims 7 to 11, wherein the binding polymers comprise polyurethane-based, acrylic-based, polyvinyl-alcohol-based, styrene-butadiene-based and/or silicone-based polymers.

13. The method according to any one of Claims 7 to 12, comprising, after the surface treatment with adhesive, a step of smoothing of the substrate, wherein the substrate is smoothed up to Bendsten ISO 2494 roughness values of less than 50 ml/min, preferably of less than 30 ml/min, and indicatively 20 ml/min.

14. The method according to any one of Claims 7 to 13, wherein the step of application of the glossy coating is performed with an air-blade or smoothing blade coating machine.

15. The method according to any one of Claims 7 to 14, comprising a step of drying of the glossy coating, conducted in an infrared oven and/or hot-air oven at a temperature of between 100°C and 180°C and with an oven time of between 0.5 and 4 minutes.

16. The method according to any one of Claims 7 to 15, comprising a step of mechanical treatment of the surface provided with the glossy coating, in particular a smoothing step and/or an embossing step.

## Patentansprüche

1. Sandraueffektpapiermaterial, umfassend ein Substrat, gebildet aus einer Mischung aus Zellulosefasern, enthaltend mindestens einen Polymerstoff, geeignet, um die Fasermischung zu verstärken, sowie einen anorganischen Füllstoff, und aufweisend mindestens eine Oberfläche, die mit mindestens einem Oberflächenkleber behandelt ist und einer Glanzbeschichtung versehen ist, gebildet aus einem oder mehreren bindenden Polymeren und/oder Wachsen, vermischt mit Pigmenten; und wobei die Pigmente Pigmente mit einer Basis aus Calciumsilikat umfassen, sodass das Papiermaterial eine sandähnliche raue Haptik besitzt, wobei die calciumsilikatbasierenden Pigmente eine variable Korngröße und einen Weißgrad aufweisen, der höher als 85 gemäß dem DIN-5033-Standard ist.

2. Papiermaterial nach Anspruch 1, wobei der Polymerstoff, der im Substrat enthalten ist, ein oder mehrere kolophoniumbasierte und/oder alkylketendimerbasierte und/oder acetylbernsteinsäurebasierte und/oder epichlorhydrinbasierte Harze und/oder modifizierte Stärken umfasst.

3. Papiermaterial nach Anspruch 1 oder Anspruch 2, wobei es sich beim anorganischen Füllstoff um einen Mineralfüllstoff handelt, der einen oder mehrere Stoffe umfasst, ausgewählt aus der Gruppe, bestehend aus Carbonaten, Kaolinen, Talk und Mischungen davon.

4. Papiermaterial nach einem der vorangehenden Ansprüche, wobei es sich beim Oberflächenkleber um einen Kleber mit einer Stärke- und/oder Polyvinylalkohol- und/oder Acryl-, Polyurethan- und/oder Styrol-Butadien-Polymer-Basis handelt.

5. Papiermaterial nach einem der vorangehenden Ansprüche, wobei die Glanzbeschichtung Pigmente mit einer lamellaren oder flachen Struktur umfasst wie z. B. gefälltes Calciumcarbonat (PCC), Kaoline für die Beschichtung, kalzinierte und/oder lamellare Kaoline, in Kombination mit den calciumsilikatbasierenden Pigmenten.

6. Papiermaterial nach einem der vorangehenden Ansprüche, wobei die bindenden Polymere polyurethanbasierte, acrylbasierte, polyvinylalkoholbasierte, styrolbutadienbasierte und/oder silikonbasierte Polymere umfassen.

7. Verfahren zur Herstellung des Papiermaterials nach einem der vorangehenden Ansprüche, umfassend die folgenden Schritte:
(a) Vorbereiten eines wässrigen Breis aus Zellulosefasern, enthaltend mindestens einen Polymerstoff, geeignet, um die Fasermischung zu verstärken, sowie einen anorganischen Füllstoff;
(b) Beseitigen des Wassers aus dem Brei, um ein Substrat des Papiermaterials zu bilden;
(c) Behandeln mindestens einer Oberfläche des Substrats mit mindestens einem Oberflächenkleber, sodass dem Substrat Eigenschaften des Wassereindringens verliehen werden, die für einen nachfolgenden Beschichtungsschritt geeignet sind; und
(d) Auftragen, auf die behandelte Oberfläche, eine Glanzbeschichtung, gebildet aus einem oder mehreren bindenden Polymeren und/oder Wachsen, vermischt mit Pigmenten, die calciumsilikatbasierte Pigmente umfassen, sodass das Papiermaterial eine sandähnliche Haptik besitzt, wobei die calciumsilikatbasierten Pigmente eine variable Korngröße und einen Weißgrad aufweisen, der höher als 85 gemäß dem DIN-5033-Standard ist.

8. Verfahren nach Anspruch 7, wobei der Polymerstoff, der im Substrat enthalten ist, ein oder mehrere kolophoniumbasierte und/oder alkylketendimerbasierte und/oder acetylbernsteinsäurebasierte und/oder epichlorhydrinbasierte Harze und/oder modifizierte Stärken umfasst.

9. Verfahren nach Anspruch 7 oder Anspruch 8, wobei es sich beim anorganischen Füllstoff um einen Mineralfüllstoff handelt, der einen oder mehrere Stoffe umfasst, ausgewählt aus der Gruppe, bestehend aus Carbonaten, Kaolinen, Talk und Mischungen davon.

10. Verfahren nach einem der Ansprüche 7 bis 9, wobei es sich beim Oberflächenkleber um einen Kleber mit einer Stärke- und/oder Polyvinylalkohol- und/oder Acryl-, Polyurethan- und/oder Styrol-Butadien-Polymer-Basis handelt.

11. Verfahren nach einem der Ansprüche 7 bis 10, wobei die Glanzbeschichtung Pigmente mit einer lamellaren oder flachen Struktur umfasst, wie z. B. Calciumcarbonat, gefälltes Calciumcarbonat (PCC), kalzinierte und/oder lamellare Kaoline, Kaoline zur Beschichtung in Kombination mit den calciumsilikatbasierenden Pigmenten.

12. Verfahren nach einem der Ansprüche 7 bis 11, wobei die bindenden Polymere polyurethanbasierte, acrylbasierte, polyvinylalkoholbasierte, styrolbutadienbasierte und/oder silikonbasierte Polymere umfassen.

13. Verfahren nach einem der Ansprüche 7 bis 12, umfassend, nach der Oberflächenbehandlung mit Kleber, einen Schritt des Glättens des Substrats, wobei das Substrat bis zu Rauheitswerten nach Bendtsen ISO 2494 von weniger als 50 ml/min geglättet wird, vorzugsweise von weniger als 30 ml/min und etwa von 20 ml/min.

14. Verfahren nach einem der Ansprüche 7 bis 13, wobei der Schritt des Auftragens der Glanzbeschichtung mit einer Beschichtungsmaschine mit Luftmesser oder Flächenspachtel durchgeführt wird.

15. Verfahren nach einem der Ansprüche 7 bis 14, umfassend einen Schritt des Trocknens der Glanzbeschichtung, durchgeführt in einem Infrarotofen und/oder einem Heißluftofen bei einer Temperatur zwischen 100 °C und 180 °C und mit einer Trocknungszeit zwischen 0,5 und 4 Minuten.

16. Verfahren nach einem der Ansprüche 7 bis 15, umfassend einen Schritt der mechanischen Bearbeitung der Oberfläche, versehen mit der Glanzbeschichtung, insbesondere einen Schritt zum Glätten und/oder einen Schritt zum Prägen.

## Revendications

1. Matériau de papier à effet sablé rugueux, comprenant un substrat, formé par un mélange de fibres cellulosiques contenant au moins une substance polymérisée, apte à donner une résistance au mélange de fibres, et une charge inorganique ; et ayant au moins une surface traitée avec au moins un adhésif de surface et pourvue d'un couchage brillant formé d'un ou de plusieurs polymères fixant et/ou d'une ou plusieurs cires, mélangés(es) à des pigments ; et dans lequel les pigments comprennent des pigments avec une base de silicate de calcium de sorte que le matériau de papier procure une sensation rugueuse semblable à du sable, les pigments à base de silicate de calcium ayant une grosseur de grain variable et un degré de blanc supérieur à 85 conformément à la norme DIN 5033.

2. Matériau de papier selon la revendication 1, dans lequel la substance polymérisée incluse dans le substrat comprend une ou plusieurs résines à base de colophane et/ou de dimère alkylcétène et/ou d'acide acétyl succinique et/ou d'épichlorhydrine et/ou d'amidons modifiés.

3. Matériau de papier selon la revendication 1 ou la revendication 2, dans lequel la charge inorganique est une charge minérale et comprend une ou plusieurs substances sélectionnées dans le groupe composé de carbonates, kaolins, talc et leurs mélanges.

4. Matériau de papier selon l'une quelconque des revendications précédentes, dans lequel l'adhésif de surface est un adhésif ayant une base d'amidon et/ou d'alcool polyvinylique et/ou d'acrylique, de polyuréthane et/ou de polymères butadiène-styrène.

5. Matériau de papier selon l'une quelconque des revendications précédentes, dans lequel le couchage brillant comprend des pigments à structure lamellaire ou plate, tels que, par exemple, le carbonate de calcium précipité (CCP), les kaolins pour couchage, les kaolins calcinés et/ou lamellaires, en combinaison avec des pigments à base de silicate de calcium.

6. Matériau de papier selon l'une quelconque des revendications précédentes, dans lequel les polymères fixant comprennent des polymères à base de polyuréthane, d'acrylique, d'alcool polyvinylique, de butadiène-styrène et/ou de silicone.

7. Procédé de fabrication du matériau de papier selon l'une quelconque des revendications précédentes, comprenant les étapes de :
(a) préparer une pâte aqueuse de fibres cellulosiques contenant au moins une substance polymérisée, apte à donner une résistance au mélange de fibres, et une charge inorganique ;
(b) retirer l'eau de la pâte pour former un substrat du matériau de papier ;
(c) traiter au moins une surface du substrat avec au moins un adhésif de surface de manière à procurer au substrat des caractéristiques d'absorption d'eau appropriées pour une étape de couchage subséquente ; et
(d) appliquer à la surface traitée un couchage brillant formé d'un ou plusieurs polymères fixant et/ou d'une ou plusieurs cires, mélangés(es) à des pigments comprenant des pigments à base de silicate de calcium de sorte que le matériau de papier procure une sensation semblable à du sable, dans lequel les pigments à base de silicate de calcium ont une grosseur de grain variable et un degré de blanc supérieur à 85 conformément à la norme DIN 5033.

8. Procédé selon la revendication 7, dans lequel la substance polymérisée incluse dans le substrat comprend une ou plusieurs résines à base de colophane et/ou de dimère alkylcétène et/ou d'acide acétyl succinique et/ou d'épichlorhydrine et/ou d'amidons modifiés.

9. Procédé selon la revendication 7 ou la revendication 8, dans lequel la charge inorganique est une charge minérale et comprend une ou plusieurs substances sélectionnées dans le groupe composé de carbonates, kaolins, talc et leurs mélanges.

10. Procédé selon l'une quelconque des revendications de 7 à 9, dans lequel l'adhésif de surface est un adhésif ayant une base d'amidon et/ou d'alcool polyvinylique et/ou d'acrylique, de polyuréthane et/ou de polymères butadiène-styrène.

11. Procédé selon l'une quelconque des revendications de 7 à 10, dans lequel le couchage brillant comprend des pigments à structure lamellaire ou plate tels que, par exemple, le carbonate de calcium, le carbonate de calcium précipité (CCP), les kaolins calcinés et/ou lamellaires, les kaolins pour couchage en combinaison avec des pigments à base de silicate de calcium.

12. Procédé selon l'une quelconque des revendications de 7 à 11, dans lequel les polymères fixant comprennent des polymères à base de polyuréthane, d'acrylique, d'alcool polyvinylique, de butadiène-styrène et/ou de silicone.

13. Procédé selon l'une quelconque des revendications de 7 à 12, comprenant, après traitement de la face avec un adhésif, une étape consistant à adoucir le substrat, dans lequel le substrat est adouci jusqu'à des valeurs de rugosité Bendtsen ISO 2494 inférieures à 50 ml/min, de préférence inférieures à 30 ml/min et de façon indicative autour de 20 ml/min.

14. Procédé selon l'une quelconque des revendications de 7 à 13, dans lequel l'étape d'application du couchage brillant est effectuée avec une coucheuse à la lame à air ou à la lame à lissage.

15. Procédé selon l'une quelconque des revendications de 7 à 14, comprenant une étape de séchage du couchage brillant, réalisée dans un four à infrarouges et/ou un four à air chaud à une température comprise entre 100 et 180 °C pendant une durée comprise entre 30 secondes et 4 minutes.

16. Procédé selon l'une quelconque des revendications de 7 à 15, comprenant une étape de traitement mécanique de la face pourvue du couchage brillant, en particulier une étape consistant à adoucir et/ou une étape de gaufrage.
